

1

3,005,710

## LATENSIFICATION OF PHOTOGRAPHIC EMULSIONS

Marilyn Levy, Red Bank, N.J., assignor to the United States of America as represented by the Secretary of the Army

No Drawing. Filed July 6, 1959, Ser. No. 825,375

5 Claims. (Cl. 96—65)

(Granted under Title 35, U.S. Code (1952), sec. 266)

The invention described herein may be manufactured and used by or for the Government for governmental purposes without the payment of any royalty thereon.

This invention relates to a method of increasing the effective speed of photographic emulsion by treating the emulsion with a dilute solution of guanidine carbonate after exposure and before development.

Several methods of increasing the useful film speed of photographic emulsions have been described in photographic literature and used in practice. Examples of such prior methods are as follows:

The use of high speed developers or extended development time; hypersensitization or treatment before camera exposure; intensification after development; and latent image intensification or latensification between exposure and development. Latensification may be accomplished by bathing the emulsion in a solution of certain chemicals, exposure to vapors or exposure to light. This invention relates to latensification by bathing.

Prior methods of latensification by bathing after exposure and before development have included certain procedural techniques which render such methods unsatisfactory. According to these prior procedures, the film must be bathed for prolonged periods and then squeegeed and dried at normal temperatures before it can be developed in the conventional manner. The inconvenience of drying film at room temperature in the dark precludes its practical utilization as a method of increasing film speed.

The present invention is based on the discovery that the effective speed of the photographic emulsion can be multiplied by bathing it in a dilute solution of guanidine carbonate after exposure and before development for a considerable time without producing an increased background fog even after several minutes of immersion. After ten minutes of immersion in the guanidine carbonate solution a background fog of only about 0.06 above normal is produced.

The invention will become more apparent from the following specific embodiments:

### Example 1

A commercial photosensitive silver halide emulsion having an ASA exposure index rating of 650 is first exposed in the camera according to the desired increased speed rate. After exposure the film is placed in a 0.5 molar aqueous solution of guanidine carbonate of the formula—



for about ten minutes. The emulsion is then developed with or without rinsing in water in a developer for about ninety seconds, for instance, in an "Eastman Kodak" de-

2

veloper known in the trade as "D-72" having the following composition:

|                                             |     |      |
|---------------------------------------------|-----|------|
| Water                                       | cc  | 500  |
| Elon (Mono-methyl paraaminophenole sulfate) | gms | 3.1  |
| Sodium sulfite (desiccated)                 | do  | 45.0 |
| Hydroquinone                                | do  | 12.0 |
| Sodium carbonate, monohydrated              | do  | 80.0 |
| Potassium bromide                           | do  | 1.9  |

10 Water to make 1.0 liter.

The film is then fixed, washed and dried.

### Example 2

A commercial silver halide film, having an ASA exposure index rating of 50 is treated as described in Example 1 using instead of a 0.5 molar solution a 2 molar solution of guanidine carbonate. The film is immersed for about one minute in this solution and then developed with or without rinsing in water for about ninety seconds at 68° F. in an "Ilford Developer" known in the trade as "ID-62" having the following composition:

|                                     |     |      |
|-------------------------------------|-----|------|
| Warm water (125° F.)                | cc  | 750  |
| Sodium sulfite (Anhyd)              | gms | 50.0 |
| Hydroquinone                        | do  | 12.0 |
| 25 Sodium carbonate (desiccated)    | do  | 60.0 |
| Phenidone (1-phenyl-3-pyrazolidone) | do  | .5   |
| Potassium bromide                   | do  | 2.0  |
| Benzotriazole                       | do  | .2   |

Water to make 1.0 liter.

30 The film is then fixed, washed and dried.

Films treated according to the present invention show an increase in speed up to about four times the speed of normal development in the above-described developers. Generally it may be said that an increase in the time of 35 immersion in guanidine carbonate results in an increase in film speed.

It will be obvious to those skilled in the art that various concentrations of the guanidine carbonate solution may be used up to about a 5 molar solution and that the time 40 of treating the film may be varied up to about twenty minutes according to the different characteristics of the exposed film and the effects desired.

### What is claimed is:

1. A method of latensification of photographic silver halide emulsions comprising treating the emulsion after exposure and before developing with an aqueous solution of guanidine carbonate whereupon the emulsion is developed in the conventional manner.
2. A method of latensification of photographic silver halide emulsions according to claim 1 in which the treatment with guanidine carbonate is continued for a time period of between one to twenty minutes.
3. A method of latensification of photographic silver halide emulsions according to claim 1 in which a 1 molar 55 solution of guanidine carbonate is used.
4. A method of latensification of photographic silver halide emulsions according to claim 1 in which a 5 molar solution of guanidine carbonate is used.
5. A method of latensification of photographic silver halide emulsions according to claim 1 in which the emulsion is treated in a 2 molar solution of guanidine carbonate for about ten minutes.

### References Cited in the file of this patent

- 65 UNITED STATES PATENTS  
60 2,165,797 Jones et al. July 11, 1939